

March 6, 1928.

1,661,416

D. ESTES

STOPPER FOR ACID BOTTLES AND PROCESS FOR MAKING THE SAME

Filed Jan. 24, 1925

*Fig. 1.*



*Fig. 2.*



*Inventor  
Dana Estes  
by Mitchell, Chadwick & Kent  
Attorneys*

## UNITED STATES PATENT OFFICE.

DANA ESTES, OF BROOKLINE, MASSACHUSETTS.

## STOPPER FOR ACID BOTTLES AND PROCESS FOR MAKING THE SAME.

Application filed January 24, 1925. Serial No. 4,534.

This invention relates to improvements in stoppers for acid bottles and processes for making the same.

More particularly it relates to the reinforcing of such stoppers when made of brittle material as for example of porcelain; and it has especial reference to the use of such stoppers in acid and alkali portable fire extinguishers. In such cases, and in any similar cases to which the invention is applicable and useful, it is desired to provide so that an accidental fracture of the porcelain is not likely to interfere with the proper function of the stopper when the apparatus is put to use.

In extinguishers of this type a canister ordinarily holding several gallons of alkali solution has in its top portion a bottle of acid, usually sulfuric, whose stopper is loosely seated and is arranged in harmony with adjacent parts so as to keep the acid and its creepage safely away from metal and alkali; but so that upon inversion of the acid container the stopper will fall to a position which permits outflow of acid from the then inverted bottle, and which to an extent regulates or controls the rate of flow. Such stoppers are usually made of porcelain, which is a brittle material liable to fracture; and although lead has been sometimes used it and other metals are objectionable as being liable to corrosion if acid gets at them. It is the purpose of the present invention to provide so that the stopper fragments will be held together if a fracture occurs, and not fall apart and lodge in such a way as to interfere with the outflow of acid when the fire extinguisher is wanted for use.

It has been proposed by me in a co-pending application for patent Serial 605,384, dealing more especially with the material steatite for manufacture of stoppers, of which this present application is in part a division, that a preventative against the separation of fragments may be had by providing a metallic core with which the earthy material of the stopper is enmeshed by structural shapes such as screw threads or flanges on the metallic element. The present invention provides an improvement upon that, available in the case of porcelain, permitting one to dispense with the screw threads or the flanges and to employ a piece of wire which is initially smooth. This core is held in place with respect to the porcelain in which it is embedded by a species of flux

therewith and resulting adsorption or micro-engagement. For this purpose nichrome wire may be used advantageously, having a coefficient of expansion which does not differ materially from that of the stopper. When such a core is inserted in the stopper during the molding of the clay, and the clay is then fired in a kiln in the usual manner, I have found that an interflux or readjustment may occur so that in the final result the porcelain adheres strongly to the wire core. It appears to me probable that the interflux is between the clay and the oxide of the metal composing the wire which forms as a coating on the metal, rather than with the metal body of the wire itself, but the exact details of this structure are extremely difficult to determine because of the microscopic nature of the dimensions involved.

It is an advantageous result of the invention that a stopper can be made for the purposes stated in which there is reinforcement by metal and yet no metal whatever is exposed to the acid; and in a preferred form indeed no metal need be exposed at all. A simple length of wire rod is set in the clay which is to become porcelain, with the porcelain at the inner end of the stopper covering deeply that end of the reinforcing rod. The other end of the rod is at the surface of the clay; but the glaze of the porcelain which is next applied covers it with a thin coat through which the end of the rod is visible. It is intended that the patent shall cover, by suitable expression in the appended claims, whatever features of patentable novelty exist in the invention disclosed.

In the accompanying drawings:

Figure 1 represents a medial section through the end portion of a portable fire extinguisher, while inverted as for use; and

Figure 2 is a medial vertical section through the lower tip end of the stopper which is seen in Figure 1, greatly enlarged.

Practice of the invention is very simple. A body of clay suitable for making porcelain when fired is prepared with a piece of suitable wire arranged axially within it, the said clay being molded into the form of a stopper and the said wire being here shown in the form of a straight rod inserted endwise, in close contact with the clay. Preferably this wire does not extend so far as to become exposed at the inner end of the axis, toward the acid. It may, however, remain exposed at the other end, which is

the top of the stopper when the apparatus is upright awaiting use, being the under part of the stopper as represented in Figure 1. If any projects after the burning it may be ground down till flush with the porcelain; and the later application and firing of the glaze makes a coating over the exposed end as seen clearly in the under part of Figure 2. The rod may be ordinary nichrome wire, which, I understand to be alloy having a high percentage of nickel alloyed with steel, to which there may be added other matter as chromium which will increase the refractory power and the resistance to chemical action, although I have not found this necessary. The wire may be, for example, from 35 to 45 one thousandths of an inch in diameter, clean and bright; and the formula for its composition may be so selected that the wire will have approximately the same coefficient of expansion as the clay or porcelain, so that during the cooling it does not break free from its engagement.

In the process of manufacture the clay is selected, mixed and otherwise treated or prepared as heretofore for the manufacture of the article and then is formed into the desired shape by the usual molding process. It is well understood that articles such as these stoppers are molded by pressure upon a body of clay between a pair of suitably shaped dies. The rod that is to be in the core of the finished stopper of the invention may be slightly longer than is portrayed at 12 in Figure 1, having its lower end, extending below the lower surface of the stopper as there seen and set into a suitable socket formed in the matrix, which thus holds the rod upright in the midst of the space which is to be filled with clay. The clay is then packed into the matrix around this rod, the top part of the die is closed over it, and the contents molded by strong pressure as usual. Being then removed and burned in a kiln as usual, the clay becomes porcelain, and a physico-chemical reaction occurs between the metal of the rod and the ingredients of the clay, as is manifest by the discoloration of porcelain and of the surface of the rod; and by the appearance of a film 16, having the nature or general aspect of a metallic oxide, between the rod 12 and the main body 10 of porcelain. On a specimen of the preferred type there appears to have been, as a result of the burning and cooling, some degree of interflux with the vitreous adjacent matter, and an adsorption upon the metallic surface. After higher temperature these effects are more marked and they are less at lower; but in either case the result is that the straight smooth wire rod has become securely engaged and held within the porcelain mass. A portion of the rod projects a little from the porcelain, being that portion which was set into the matrix; and this can be cut off with nippers

pers and then ground down till it is flush with the surface of the porcelain. Then the application of glaze and its subsequent burning will cover the end of the rod together with the porcelain as shown by the hard glaze 14 at the lower part of Figure 2, covering the end of the rod. It is to be observed, however, that no particular defect in the finished article would be recognized even though the glaze did not cover the outer end of the rod.

Figure 2 shows on a greatly enlarged scale, more or less diagrammatically, the porcelain 10, the nichrome wire 12, and the intervening engaging film 16 which the wire rod is believed to have adsorbed on its surface, the interflux being indicated by the irregular line forming the boundary between the part 16 and porcelain 10. It is important to regulate the flow of the fire extinguishing fluid through the discharge 20, as is already well known. If a finished stopper becomes broken the central rod will hold in place any parts which encircle the rod. And if in some places it should happen that the interflux has not been perfect as above described so that at those places the fragment is loose upon the rod, nevertheless the holding of the rod at the other places will hold the loose piece in place and thus will maintain the predetermined size of opening for exit of the acid to mix with alkali, seen in Figure 1 at 18.

I claim as my invention:

1. The combination, with an invertible fire extinguisher having an acid bottle, of a loose stopper for the bottle, subject to concussion within the extinguisher when the extinguisher is inverted and means to maintain the material thereof in stopper formation notwithstanding its fracture; said stopper comprising a body of vitrified earthy material; and said means comprising a rod, made of metal whose coefficient of expansion is close to that of said earthy material, penetrating said material and arranged in intimate clinging contact therewith, whereby fracture of the stopper is resisted, and there is a tendency of the fragments, if fracture occurs, to be held in the stopper formation by the said rod.

2. The combination, with an invertible fire extinguisher having an acid bottle, of a loose stopper for the bottle subject to concussion within the extinguisher when the extinguisher is inverted, and means to maintain the material thereof in stopper formation notwithstanding its fracture; said stopper comprising a body of porcelain; and said means comprising a rod made of metal whose coefficient of expansion is substantially the same as that of the porcelain, penetrating said porcelain; there being an interflux between the porcelain and said rod whereby fracture of the stopper is resisted, and there

is a tendency of the fragments, if fracture occurs, to be held in the stopper formation by the said rod.

3. A bottle stopper made of vitrified earthy material and having enclosed entirely within it a rod of metal whose coefficient of expansion is substantially the same as that of the said material; said material being in

intimate and clinging contact with the surface of said rod, whereby fragments of a fractured stopper cling to the rod and by it are held together.

Signed at Boston, Massachusetts, this twenty-second day of January, 1925.

DANA ESTES.